

April 2, 1929.

L. R. MacKENZIE

1,707,939

WEAR COURSE FOR PAVEMENTS

Filed Aug. 6, 1928

2 Sheets-Sheet 1

Fig. 1.



Fig. 2.



Fig. 3.



Inventor

Leon R. MacKenzie

by Bair, Freeman & Sinclair  
Attorneys

Witness

Dave Bair

April 2, 1929.

L. R. MacKENZIE

1,707,939

WEAR COURSE FOR PAVEMENTS

Filed Aug. 6, 1928

2 Sheets-Sheet 2



Inventor  
Leon R. MacKenzie  
by Bair, Freeman & Sinclair  
Attorneys

Witness  
David Bair

## UNITED STATES PATENT OFFICE.

LEON R. MACKENZIE, OF DES MOINES, IOWA.

## WEAR COURSE FOR PAVEMENTS.

Application filed August 6, 1928. Serial No. 297,633.

My invention has to do with a wear course for a pavement of the asphalt or bituminous type.

It is my purpose to provide a pavement so constructed by simple and economical methods that the normal movement of the body of material within itself is prevented or eliminated.

It is also my purpose to provide a simple and inexpensive method of making such a pavement.

With these and other objects in view, my invention consists in the arrangement and construction of the pavement and the method 15 of making the same as set forth in the following description defined in my claims, and illustrated in the accompanying drawings, in which:

Figure 1 shows a perspective view, partly 20 in section, of the lower course, re-inforcing and upper course of my pavement before they are placed in proper superposed position.

Figure 2 shows a vertical, sectional view 25 of the pavement, illustrating it before and after rolling.

Figure 3 is a perspective view of a piece of the mesh re-inforcing.

Figure 4 is a perspective view, partly 30 in section, of the pavement, illustrating the relative arrangement of courses and re-inforcing.

Figure 5 is a vertical, sectional view of the pavement made in one way, before rolling.

Figure 6 is a similar view of the same 35 pavement after it is rolled.

Figure 7 is a vertical, sectional view of the pavement laid in a slightly different way, before rolling; and

Figure 8 is a similar view of the same, 40 after rolling.

Highway engineers recognize generally that the sheet asphalt type makes perhaps the most satisfactory top or wearing course 45 for a pavement surface. The asphaltic top or wearing course is laid upon a suitable base, such as rolled gravel, concrete, bituminous mixture, water-bound macadam and so on.

Heretofore the use of sheet asphalt for the 50 wearing course of the pavement has been subject to recognized difficulties and defects.

It has been extremely difficult to prevent the somewhat plastic asphalt or bituminous layer from shifting or rolling to form high and 55 low spots, which cause rough traffic surface conditions.

The use of motor vehicles has greatly increased these difficulties. The effect of stopping and starting of motor vehicles and general motor vehicle traffic tends to pull or push the upper portion of the asphalt coat or surface, forming the ridges, humps and hollows which are so well known.

It is well known that during the summer 65 months when the air temperature is quite high that asphaltic materials, from which the wear course of a pavement is ordinarily formed, are subjected to easy displacement due to traffic upon the wear course.

The asphaltic materials during the high 70 temperature of the summer months are comparatively soft or pliable and due to traffic thereon are very quickly and easily displaced.

It is further well known that asphaltic materials have a greater affinity for heat and the retention of the same. It thus follows that the heat which is absorbed within the pavement will give to the pavement a temperature 80 greater or higher than the air temperature.

The degree of heat within the pavement is retained for a considerable length of time 85 after the sun's heat rays have been absorbed, and it is my object to provide a pavement that will eliminate the movement of the asphaltic material within itself.

When the surface material does move until the surface course is of different thicknesses at different places, the wear and deterioration subsequently increase rapidly. Small depressions and then holes develop in the surface, which are enlarged by continuous pushing, shoving and traffic impact and traction, resulting in the formation of more 95 humps, ridges and hollows and ultimate exposure of the base in places. When the holes are so formed or the base exposed, water works into the holes and low places, seeps under the surface sheet, and increases the 100 rapidity of disintegration of the entire paving.

These difficulties have been largely accredited to the separation of the top course from

the base, and many devices, structures and methods have been employed for anchoring the top course to the base with varying degrees of success.

5 I have found due to increase of motor transportation that the difficulties heretofore experienced are largely due to the fact that the so-called or commonly known bituminous or asphaltic top course has movement 10 within itself. That is to say, the upper portion thereof moves with relation to the lower portion, somewhat as in the case of a layer of soft chewing gum, the upper portion of which could be pushed about and would thus 15 move with relation to the lower portion, even though the lower portion might be fixed to a base.

I have found that there is in any bituminous pavement course, what may be called an 20 axis of movement within itself. Even though the lower part of the course may be anchored to the base, the upper part of the plastic material will move with relation to the lower part. On approximately an inch in 25 thickness of rolled surface asphalt under traffic, this axis of movement is scarcely perceptible, at approximately an inch and a half it becomes apparent, and over two inches it is quite noticeable.

30 The various methods and structures which have been adopted for anchoring the asphaltic top course to the base course have therefore been unsatisfactory because they did not prevent the rolling or movement of the upper 35 part of the asphaltic course within itself, and the resultant wavy formation causing a rough traffic surface unsatisfactory for traffic and leading to more rapid deterioration.

Under present traffic conditions, a bituminous 40 course, which is thin enough to eliminate this normal movement of the material within itself, is too thin for practical use.

A relatively thin asphaltic or bituminous course is not sufficient for practical purposes, 45 due to the fact that it will not stand weather and traffic conditions to which it is generally subjected. Such asphaltic courses usually have from seven to ten percent of pure asphaltic or bituminous cement, containing 50 volatile oils. Hence, when a shallow body of asphalt or bituminous top mixture is exposed to the sun, there is not sufficient depth or body to the mixture to retain its vitality and wearing qualities for a proper length of time. 55 The hot summer sun in time will draw out the volatile oils, and there remains a hard coke-like substance, which quickly disintegrates and pulverizes under traffic.

It therefore follows that where there is not 60 sufficient depth to the asphalt wearing course mixture, its life and wearing qualities are too greatly reduced, whereas if the course is of sufficient thickness to retain the volatile matter, which lends life to the surface, the thickness 65 is great enough so that there is in the

body a normal movement under traffic which results in rough surface and subsequent rapid disintegration.

Practice has not yet proven the solution of the problem. If the sheet of asphaltic or bituminous mixture is lowered in depth sufficiently to overcome the normal movement within itself, it then becomes too shallow to give long life to the pavement, and if the depth is sufficiently increased to retain the 70 chemical ingredients essential for prolongation of the life of the material, the axis of movement within itself is far enough below the top of the surface to permit movement 75 above that axis with the resultant rolling 80 and wave-like formation, which is highly objectionable.

It is obvious that anchoring the top course to the base will not meet these objections.

Efforts have been made by the admixture 85 of certain hardening chemicals to make the asphalt sufficiently rigid not to move within itself and at the same time to leave it sufficiently plastic, so that at cold temperatures when hardening takes place, there will be 90 sufficient flexibility to avoid the breaking and disintegration of the surface. These mixtures, however, have not yet proven efficient to remedy the evil.

I have therefore in my present invention 95 provided a pavement wearing course construction, whereby the axis of movement within the body of plastic material is so raised as to permit it to be negligible in an asphaltic or bituminous top course of sufficient thickness to retain its volatile oils and proper longevity and utility as a pavement.

My pavement may be laid upon worn-out concrete pavement, which has to be re-surfaced, or upon water-bound macadam base, 105 rolled gravel base, or bituminous mixture base, or any other bases of sufficient stability to act as such.

I shall describe two slightly different methods of constructing my pavement. These 110 methods involve the same general thought and principle and produce a pavement wear course accomplishing my purpose of so anchoring the upper and lower layers of the body of plastic surface material that the axis of movement is practically eliminated or becomes a negligible factor.

According to the first method, as shown in Figure 1, I place upon the base 10 a course A of asphaltic concrete or bituminous mixture, containing standard materials, for which I suggest, for example, approximately seven percent of pure asphalt cement, fine sands, and hard crushed rock or stone 12, sized from one to one and one-fourth inches in greatest dimension.

The mixture may be placed on the base while hot to a uniform thickness of not less than approximately one inch, so that it will be approximately three-fourths of an inch in 130

depth. I suggest about seventy pounds of mixed material to the square yard.

This layer should be raked or fluffed uniformly in the ordinary way to the true contour of the base.

After raking, I place on top of this layer, sheets of expanded metal (steel) reinforcement 14 having openings of approximately two to two and one-half inches in their long dimensions (inside measurement) and approximately one to one and one-half inches in their short dimensions (inside measurement). This mesh can be readily placed by hand and the edges merely interlocked to make a continuous mat or mesh over this whole lower course of asphaltic material.

As soon as possible another similar course or layer B is placed above the bottom course with the mesh thereon. The whole mass is then rolled. The rolling causes the stones in the mixture to protrude up from the bottom course or project down from the top course or both through the mesh of steel, thereby interlocking themselves in the upper and lower portions or layers of asphaltic material, through this semi-rigid steel center plane, and thus tying the whole mass completely and effectively together, and raising the axis of movement, which would ordinarily be about the level of the steel to somewhere near the top of the inch over and above the steel, where it will be negligible.

Thus in Figure 2, I have shown the pavement at the left, before rolling by the roller 16, and at the right, after rolling. The pavement before rolling is also illustrated in Figure 5 and after rolling in Figure 6.

The relative size of the openings in the mesh and of the stone should be such that when the compression of the pavement has occurred and the stone pressed closely together in the mass, there can be no movement of the upper portion of the pavement sufficient to cause harmful results because of the anchorage afforded by the arrangement of the stone with relation to the mesh and the asphaltic mixture above and below it.

Upon final completion, it would only be necessary to use a paint coat or a squeegee coat of hot asphalt cement over the surface and sand it down by brooming hot clean sand over the paint or seal coat of asphalt.

The result under traffic after the original seal coat has been worn down is a monolithic surface containing high stone content meeting the abrasion and wear, thoroughly keyed to a semi-rigid steel mesh anchored in the center of the surface slab by larger stone protruding both upward and downward through the mesh. Thus there would not be permitted any substantial movement of any one stone under traffic to move it further than a small portion of the mesh opening in the steel itself.

Inasmuch as the stone would be approxi-

mately of a size to wedge itself into the mesh opening, it would be impossible for the stone to move to any degree to form in the plastic surface rolls or surface imperfections to any extent which would be noticeable to traffic.

The alternative slightly different method for making this pavement is as follows:

There is placed upon the base a course of sheet asphalt or bituminous material 18, containing no large aggregate, of such a thickness that if rolled it will not be less than three-fourths of an inch in depth. (Figure 7.) This should be raked or fluffed to a true contour.

After raking, there is placed on this layer of sheet asphalt, expanded sheet metal 14, such as above mentioned.

After placing the reinforcement in position, another similar layer of asphalt mixture 20 is laid on the mesh and lower course, approximately one inch thick. This should be fluffed and may be lightly rolled or not, as practice will denote. In either case, while the mass is ready for either preliminary or final rolling, as the case may be, crushed angular hard stone or rock 22 of approximately from one to one and three-fourths inches in largest dimensions, preferably previously treated with naphthene or light oil to clean it, is cast evenly over the surface of the mass.

Immediately thereafter, the pavement is rolled with heavy rollers and thereupon the stone in the completed wear course will form a hard almost rock top surface and the larger stones or rocks will be forced down into or through the steel mesh for anchoring the bottom and top layers and steel mesh and thoroughly locking them together in the same way as has already been mentioned.

It may perhaps be stated that natural rock asphalt or cold prepared mixes may be used for my pavement as well as any of the mixtures now used or to be developed in practice.

In the completed product, if the mesh and stone are of the proper size and the two layers are of the proper thickness, the normal movement of the body of material within itself will be eliminated.

When this result has been accomplished, no anchorage of the completed top coat or course to the base is necessary. For if there is no movement in the top course itself, there will be no movement of the base. This is of particular importance in laying my pavement as a top course on old concrete pavements which have smooth surfaces and to which it would be difficult to anchor the top or wear course.

The reinforcing should preferably be substantially flat or in sheets so that it will not interfere with the raking and fluffing.

It will be noted that my pavement may be made of materials, which are generally and readily available and laid with the equipment now in general use or available.

In my claims, I intend by the use of "asphalt" or "asphaltic bitumin" or "bituminous" to include any plastic paving material adaptable for the purpose, and normally having movement within itself. Likewise by "mesh reinforcing", I would include any material suitable for my object.

I claim as my invention:

1. A pavement comprising a suitable base 10 and a wear course thereon comprising a lower asphalt layer, a metal mesh reinforcing laid thereon, an upper asphalt layer, said wear course having crushed hard rock projecting into and through the meshes of the reinforcing, the rock being of such size relative to the thickness of the course and the size of the openings in the mesh that when the wear course is compressed the rock will enter and project through and nearly fill the meshes so 15 that the two layers and reinforcing will be thoroughly anchored together.
2. A wearing course for a pavement having a lower asphaltic layer, a semi-rigid mesh anchoring element thereon, an upper asphaltic layer resting upon said lower layer and covering said anchoring element, said layers 20 having aggregate therein projecting through

the meshes of the anchoring element, said aggregate being of a maximum dimension greater than the thickness of either layer and 30 the size of the meshes being such as to receive the aggregate so that the aggregate will have substantially no horizontal movement therein.

3. A pavement comprising a course of asphaltic material, angular rock aggregate in said course of a largest dimension greater than half the thickness of the course, and means in the course substantially spaced from the top and bottom thereof for permitting movement of the rock vertically in the course when the course is compressed by traffic or otherwise and for substantially preventing the movement in a horizontal direction of that portion of the aggregate adjacent to it. 45

4. In a pavement wear course, a layer of asphaltic material, semi-rigid mesh anchoring means thereon, a top layer of asphaltic material, and hard aggregate in said course, projecting through the meshes of the anchoring means, and of a size relative to such meshes, to substantially fill them. 50

Des Moines, Iowa, July 30, 1928.

LEON R. MACKENZIE.